

## UNITED STATES PATENT OFFICE

RICHARD MICHEL, OF UERDINGEN, NIEDERRHEIN, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## INSULATING OIL

No Drawing. Application filed July 12, 1928, Serial No. 292,328, and in Germany July 16, 1927.

The invention relates to insulating oils in particular to transformer and switch oils.

Insulating oil especially transformer oil has two principal functions—(1) To act as an insulating medium, and (2) to carry the heat generated in the windings and core of the transformer or other circuits to the cooling surfaces.

This double function involves that insulating oils have to meet particularly high operating conditions. In order to warrant insulating properties answering all requirements of practice, their dielectric strength is not permitted to fall below a minimum and in order to have a good cooling effect, the viscosity dare not exceed a maximum. It is further necessary to select an oil extremely stable to increased temperature and to oxidation.

Hitherto mineral oils of suitable properties have been almost exclusively used as insulating oils. According to their geographical origin and according to the special mode of preliminary treatment (refining etc.) they vary within wide limits and tend to undergo detrimental alterations which become evident during the use of such oils.

I have found that alkylated hydrocarbons of the naphthalene series and their derivatives are excellent insulating oils in particular transformer and switch oils. Especially those hydrocarbons of the naphthalene series have been found suitable which have several side chains and the saturated side chains of which contain two and more carbon atoms.

In addition to these alkyl groups one or more methyl groups may also be present in the molecule. Derivatives of alkylated hydrocarbons of the naphthalene series such as hydrogenated naphthalene hydrocarbons or alkylated naphthalene compounds which are substituted by chlorine in the aromatic nucleus likewise may be used. A considerable number of compounds showing the aforesaid

chemical characteristics can be prepared and it is necessary to select among them those liquid compounds that will have a specific gravity sufficiently below 1 and a vapor tension sufficiently low as to answer the requirements prescribed for flash point, constance in weight and other physical characteristics. On the other hand the oils are desired to be distillable under reduced pressure.

The new insulating oils have a constant chemical composition and their physical characteristics, therefore, are also constant. By choosing appropriate compounds, the properties may be easily adapted to the special operating conditions of particular cases. The dielectric strength of the oils is considerably high and does not substantially decrease in the service. The well known testing methods and practical use indicate an extraordinary resistance to thermal and oxidizing influences, for example the tendency to form deposits known as sludge is slight and formation of acids by oxidation only takes place to an almost negligible extent which is shown by a Kissling test mostly being below 0.1 (German testing method known as "Verteerungszahl"). The oils unite a viscosity within the right limits and a very deep pour point which is frequently below  $-20^{\circ}$  C. They, too, are free from any ingredients insoluble in benzene such as asphalt and other detrimental constituents and are miscible with other appropriate oils e. g. mineral oils.

In order to give examples of the new insulating oils I name the oily products which are obtained by reacting with olefines or gases containing olefines in the presence of a catalyst upon naphthalene or homologues of naphthalene e. g. methyl naphthalenes, partially hydrogenated naphthalenes e. g. tetrahydronaphthalene, naphthalene hydrocarbons being substituted by chlorine in the nucleus e. g.  $\alpha$ - or  $\beta$ -chloronaphthalene ar-chloro tet-

rahydronaphthalene etc.; but I wish to be understood that alkylated naphthalene compounds resulting from other processes are likewise suitable as insulating oils.

5

*Example 1*

An oil which consists of a mixture of polyethyl naphthalenes boiling at 12 mm pressure from about 160 to 200° C. and having a composition of about 90 percent C and about 10 percent H, has the following properties:

Specific gravity..... 0.950  
Flash point (in an open crucible)..... 150° C.  
Pour point..... below -30° C.  
Viscosity (at 20° C.)..... 3.14° (Engler)  
Asphalt content..... 0  
Water content..... 0  
Acid number..... 0.05  
20 Kissling test (German testing method "Verteerungszahl")..... 0.07  
Dielectric strength..... 188000 volt/cm

The term "188000 volt/cm" means that an E. M. F. of 188,000 volt is necessary to cause an electric spark between two electrodes, the distance between the electrodes being 1 cm and the medium between the two electrodes being the insulating oil, the use of which is recommended in the above given example.

30

*Example 2*

An oil which consists of a mixture of polypropyl naphthalenes boiling at 12 mm pressure from about 160° to 200° C. and having a composition of about 90.5 percent C and 9.5 percent H, has the following properties:

Specific gravity..... 0.930  
40 Flash point..... 166° C.  
Pour point..... below -20° C.  
Viscosity (at 20° C.)..... 7.35° (Engler)  
Asphalt content..... 0  
Water content..... 0  
45 Acid number..... 0.04  
Kissling test (German testing method "Verteerungszahl")..... 0.06  
Dielectric strength..... 140000 volt/cm

50 An oil of similar properties obtained by reacting with propylene in the presence of aluminium chloride upon ar-chlorotetrahydronaphthalene has a dielectric strength of 165000 volt/cm.

55

*Example 3*

An oil which consists of a mixture of ethylated naphthalenes and naphthalenes substituted by higher alkyl groups, prepared by 60 reacting upon naphthalene in the presence of aluminium chloride with waste gas from cracking operations (containing about 23 percent of ethylene and 12 percent of higher homologues thereof), and boiling at 12 mm. pressure from about 160 to 200° C. and having

a composition of about 91 percent C and 9 percent H, has the following properties:

|                                                               |                |
|---------------------------------------------------------------|----------------|
| Specific gravity.....                                         | 0.948          |
| Flash point.....                                              | 148° C.        |
| Pour point.....                                               | below -25° C.  |
| Viscosity (at 20° C.).....                                    | 3.7° (Engler)  |
| Asphalt content.....                                          | 0              |
| Water content.....                                            | 0              |
| Acid number.....                                              | 0.05           |
| 20 Kissling test German testing method "Verteerungszahl"..... | 0.09           |
| Dielectric strength.....                                      | 159000 volt/cm |

70 *Example 4*

A mixture which contains equal proportions of a mineral oil (characteristics I) and the oil of Example 3 has the properties given below II:

|                                                                 | I             | II             |
|-----------------------------------------------------------------|---------------|----------------|
| Specific gravity.....                                           | 0.879         | 0.914          |
| Flash point.....                                                | 165° C.       | 155° C.        |
| Pour point.....                                                 | below -18° C. | below -20° C.  |
| Viscosity (at 20° C.).....                                      | 4.3°          | 4.1° (Engler)  |
| Asphalt content.....                                            | 0             | 0              |
| Water content.....                                              | 0             | 0              |
| Acid number.....                                                | 0.08          | 0.06           |
| 20 Kissling test (German testing method "Verteerungszahl")..... | 0.07          | 0.08           |
| Dielectric strength.....                                        | 110000        | 135000 volt/cm |

80 In the following claims the term "polyalkylated naphthalene hydrocarbon compound" is used to denote a naphthalene, a homologue thereof, and naphthalene derivatives hydrogenated and/or halogenated in at least one aromatic nucleus, having several aliphatic side chains, either singly or in admixture.

90 I claim:

1. An insulating oil comprising a liquid polyalkylated naphthalene hydrocarbon compound.
2. An insulating oil comprising a liquid polyalkylated naphthalene hydrocarbon compound having a specific gravity below 1.
3. An insulating oil comprising a liquid polyalkylated naphthalene hydrocarbon compound having a specific gravity of from about 0.850 to about 0.950.
4. An insulating oil comprising a liquid polyalkylated naphthalene hydrocarbon compound having saturated side chains with at least two carbon atoms.
5. An insulating oil comprising a polyalkylated naphthalene hydrocarbon compound having a specific gravity of about 0.950, a viscosity (at 20° C.) below 8° (Engler) a flash point above 140° C. and a pour point below -20° C.
6. A composition of matter comprising an insulating oil containing a substantial proportion of a polyalkylated naphthalene hydrocarbon compound.
7. A composition of matter comprising an insulating oil containing a substantial proportion of a polyalkylated naphthalene hydrocarbon compound having a specific gravity below 1.
8. A composition of matter comprising an insulating oil containing a substantial proportion of a polyalkylated naphthalene hydrocarbon compound having a specific gravity from about 0.850 to about 0.950.

75

80

85

90

95

100

105

110

115

120

125

130

9. A composition of matter comprising an insulating oil containing a substantial proportion of a polyalkylated naphthalene hydrocarbon compound having saturated side chains with at least two carbon atoms.
- 5 10. A composition of matter comprising a mineral oil containing a substantial proportion of a polyalkylated naphthalene hydrocarbon compound.
- 10 11. An insulating oil comprising a liquid naphthalene hydrocarbon compound which is substituted by at least two alkyl groups having at least two carbon atoms.
- 15 12. An insulating oil comprising a liquid naphthalene hydrocarbon compound which is substituted by at least two alkyl groups having 2-3 carbon atoms.
- 15 13. An insulating oil comprising a liquid naphthalene hydrocarbon compound having 20 at least two saturated side chains with 2-3 carbon atoms.
- 20 14. A composition of matter comprising an insulating oil containing a substantial proportion of a liquid naphthalene hydrocarbon compound which is substituted by at least two alkyl groups having at least two carbon atoms.
- 25 15. A composition of matter comprising an insulating oil containing a substantial proportion of a liquid naphthalene hydrocarbon compound which is substituted by at least two alkyl groups having 2-3 carbon atoms.
- 20 16. A composition of matter comprising an insulating oil containing a substantial proportion of a liquid naphthalene hydrocarbon compound having at least two saturated side chains with 2-3 carbon atoms.

In testimony whereof I have hereunto set my hand.

40

RICHARD MICHEL.

45

50

55

60

65